

Jan. 12, 1960

W. W. GULLETT

2,920,957

ALLOYS OF TITANIUM-GROUP METALS

Filed June 20, 1957

3 Sheets-Sheet 1

*Fig. 1.*



*Fig. 2.*



*Fig. 3.*



*Fig. 4.*



Jan. 12, 1960

W. W. GULLETT

2,920,957

ALLOYS OF TITANIUM-GROUP METALS

Filed June 20, 1957

3 Sheets-Sheet 2

*Fig. 5.*



*Fig. 6.*



*Fig. 7.*

Jan. 12, 1960

W. W. GULLETT

2,920,957

ALLOYS OF TITANIUM-GROUP METALS

Filed June 20, 1957

3 Sheets-Sheet 3

Fig. 8.



# United States Patent Office

2,920,957

Patented Jan. 12, 1960

1

2,920,957

## ALLOYS OF TITANIUM-GROUP METALS

William W. Gullett, College Park, Md., assignor to Chicago Development Corporation, Riverdale, Md., a corporation of Delaware

Application June 20, 1957, Serial No. 666,841

7 Claims. (Cl. 75—175.5)

The present invention relates to titanium alloys and zirconium alloys, and is concerned with the provision of titanium alloys and zirconium alloys of high strength and good ductility which alloys contain relatively small contents, only, of beta stabilizing elements.

It has been known to make titanium alloys having high strength and reasonable ductility by the addition to titanium of beta stabilizing elements such as vanadium and manganese together with at least one alpha stabilizer such as oxygen or aluminum. By suitable heat treatment, such alloys are obtained with desired proportions of alpha and beta phases. The importance of the two phases is not only to provide a dual structure, but more importantly to reduce the oxygen content of the beta phase by providing an "oxygen sink" of alpha phase, in which latter oxygen is much more soluble than it is in the beta phase. This reduction in oxygen content reduces brittleness in the beta phase.

Heretofore, in order to obtain alloys in which the beta phase is sufficiently stabilized to provide a major proportion of beta after annealing at, say, 800° C. and furnace cooling, it has been necessary to add considerable amounts of the beta stabilizing elements. Examples of such commercial titanium alloys are: 15% V, 2% Al; 6% Al—4% V; 8% manganese; 4% manganese—4% aluminum.

I have discovered that the employment of relatively large amounts of the beta stabilizing elements—heretofore necessary—has been rendered essential because the titanium (or, zirconium) "base" of the alloy as conventionally made has contained a relatively large amount of oxygen in interstitial solid solution. That is to say, I have discovered that a titanium alloy containing only a very minute amount of oxygen requires very much less of the beta stabilizer than conventionally thought necessary in order to confer thereto the desired hardness and strength properties.

My invention, therefore, consists in reducing the oxygen content of the titanium alloys to such an extent that the beta phase can be substantially stabilized with a much lower percentage of the beta stabilizing elements than heretofore known or used. As beta stabilizing agents, I may use vanadium, iron, chromium, manganese or molybdenum.

The degree of strengthening which I obtain in the beta phase before separation of alpha phase is much greater than has heretofore been obtained. One embodiment of my invention, therefore, consists in providing stable alloys entirely or substantially all beta phase, strengthened almost entirely by solution hardening of the beta phase without loss of ductility by heat treatment which is characteristic of the beta phase alloys of the prior art.

It must be pointed out for the full understanding of my invention that the critical compositions of the alloys of my invention especially as regards oxygen content refer to the fully fabricated alloy and to the specific portion of the alloy being tested. I am familiar with the practice of making alloys from pure "iodide" titanium which may have oxygen contents within the limits of

2

my invention. Such alloys in the fully fabricated form have not, in the known art, been within the composition range of my invention. This situation clearly prevails even though the investigators have not reported it and have therefore, in certain instances, given the incorrect impression that the alloys which they prepared and fabricated from iodide titanium had oxygen contents in the range of the base titanium used. The literature is replete with references showing that such an assumption is invalid. I shall here refer to only a few.

Second Progress Report on Research and Development on Titanium Alloys, Battelle Memorial Institute, October 31, 1949, Contract No. 33(038)3736, Wright Patterson Air Force Base, Dayton, Ohio, p. 116. Shows that melted iodide titanium analyzed .041 oxygen.

Summary Report on Diffusion of Hydrogen, Nitrogen, and Oxygen in Titanium, Columbia University, Report W.A.L. 401/149-112, dated July 13, 1953, to Watertown Arsenal Laboratory. Shows that iodide titanium used contained .011% oxygen but that oxygen was taken up very rapidly so that alloys fabricated by hot rolling would have oxygen contents beyond the limits of the present invention.

An illustration of the difference between the alloys of my invention and those of the prior art may be seen from the paper "Effect of Alpha Solutes on the Heat Treatment Response of Ti—Mn Alloys" by H. R. Ogden, F. C. Holden and R. I. Jaffee, Trans. A.I.M.E., January 1955, p. 105. The alloys reported on by these investigators were made from iodide titanium but were forged at 875° C. and swaged at 750°. Such a procedure raises the oxygen content beyond the limit of my invention as shown by the hardness data in Figure 12 of the paper. The hardness on furnace cooling the alloys is only about 200 Vickers at 3% manganese as compared to 412 for a 3% manganese alloy of my invention heat treated in the same manner. Clearly, a conventional hot working procedure produces fabricated alloys outside the composition limits of my invention even if highly pure iodide titanium is used as initial material.

It is very tedious and time consuming to fabricate hard strong alloys by cold work and repeated vacuum annealing. I have found that titanium carbide coatings permit hot working without oxygen absorption beyond the limits of my invention. This method is highly useful in the commercial application of my invention and is illustrated in Example IX hereinbelow.

Even when hot working was not employed, alloys of the prior art fabricated from iodide titanium have not been within the composition limits of my invention; for example, Finlay and Snyder in their article on Effects of Three Interstitial Solutes, Trans. A.I.M.E., 188, p. 277 (1950). The graphs of this report indicate values for alloys down to zero oxygen; however, these investigators analyzed only one alloy and in this found .03% oxygen above the reported values.

It may, therefore, be concluded that all the alloys reported by these investigators were outside the limits of the present invention, a conclusion fully supported by the extrapolated hardness of the base titanium of more than 100 Vickers, although the hardness of the base iodide titanium used is given as Vickers 60-70.

The unusual and unexpected results flowing from drastically reducing the content of oxygen in the titanium and zirconium alloys in accordance with my invention will be illustrated in the case of titanium-vanadium. By reducing the oxygen content, in the fabricated material, to about .01%, I make titanium-vanadium alloys up to at least 4% vanadium which are stable substantially beta alloys even when slowly cooled from 900° C. Figure 1 shows the hardness curve of these very low oxygen

titanium-vanadium alloys of my invention, the abscissæ numerals representing Vickers hardness values.

I find that a very small content of oxygen—0.01–0.03%—increases hardness probably by producing a dispersion of sub-microscopic alpha particles; however, an increase into the range of oxygen content of alloys of the prior art, that is .04–.15% oxygen, greatly lowers hardness and strength. Figure 2 shows a series of curves relating Vickers hardness to oxygen content for fabricated titanium-vanadium alloys containing from 1–4% vanadium. The peaks in hardness in the range from .01–.03% oxygen have not been heretofore known, and every expectation would have been that the hardness curves would simply extend to zero along the .15% oxygen to .06% oxygen path. My invention cannot, therefore, be considered merely the expected or conventional result of increasing purity of the alloys, but rather the unpredictable result flowing from drastically reducing the oxygen content of the alloys.

The ductility of the alloys of my invention is illustrated in the following table, which shows that the hardening and strengthening effect brought about by my invention is obtained without the conventional loss of ductility.

TABLE

| Percent V | Elong. Percent in 2" | Yield Strength |
|-----------|----------------------|----------------|
| 1.....    | 40                   | 125,000        |
| 2.....    | 30                   | 140,000        |
| 3.....    | 20                   | 170,000        |
| 4.....    | 15                   | 185,000        |

Manganese and molybdenum alloys follow the pattern of the vanadium alloys discussed in detail. The hardness curves for titanium alloys of manganese and of molybdenum are shown in Figure 3 and Figure 4, respectively, the oxygen contents in both instances being about 0.01% in the fabricated material. Ductility is slightly less for the same strength for manganese and molybdenum alloys than for the vanadium alloy.

My invention is also applicable to zirconium alloys in the same way as for titanium. Figure 5 shows the hardness curves for a zirconium-vanadium alloy containing about 0.01% oxygen in the fabricated form.

My invention has particular applicability to titanium (and, zirconium)-iron alloys, since the effect of iron on the hardness and strength of titanium (and, zirconium) is very great at the low oxygen levels referred to above. This has not, to my knowledge, been known before my invention. In Figure 6, I have plotted the yield strength and elongation of titanium-iron alloys as determined on alloys containing .06% oxygen and for alloys within the composition range of my invention, viz. .02% oxygen, all after cold reduction of 50% and annealing at 700° C.

The data which I have determined for .06% oxygen is substantially in accord with that given in McQuillan and McQuillan, "Titanium," p. 345. It is stated in that text that the titanium used to make the alloys was of high purity, however, the melting and fabricating must have introduced about .06% oxygen, since the hardness of the metal without iron is given as Brinell 100, and furthermore, the hardness at 0.5% iron was about 140 which is in good agreement with a hardness of about 150 obtained by McKinley on adding 0.5% iron to titanium containing .06% oxygen, as set forth in an article on "Effect of Impurities on the Hardness of Titanium" by T. D. McKinley, "Journal Electrochemical Society," October 1956, p. 563.

It is significant that in studying the beta stabilizing elements, iron, chromium, vanadium, molybdenum and manganese, McKinley did not report the increase in hardening effect due to beta stabilizing elements when oxygen is lowered below .06%, which is the essence of the present invention.

In Figure 6, I have plotted the yield strength and elongation for fabricated low iron alloys because these are the most important engineering parameters. It will be noted that with less than .5% iron and .02% oxygen, a yield strength can be obtained as high as with 15% iron and .06% oxygen. Further, the ductility of the low oxygen alloy is much higher at equal yield strength.

In the case of zirconium alloys, the great strengthening effect of iron is of great importance. Zirconium with .02% oxygen and .3% iron has U.T.S. 180,000 lbs., Y.S. 165,000 lbs., elongation % in 2" 20, after 50% cold reduction and annealing at 700° C.

The alloys of my invention are thermally stable in the sense that they may be reheated and furnace cooled from 700–800° C. without change. The fabricated alloys with less than .01% oxygen are not significantly hardened by quenching from 900° C., but those with .03% oxygen are hardened by as much as 100 points Brinell by such treatment. The properties are restored by annealing at 700–800° C. By long heating at 600° C., the furnace cooled alloys of my invention are not changed in hardness.

The behavior of fabricated alloys made in accordance with my invention when the content of alloying element is substantially increased is shown in Figure 8. In this figure, I have plotted yield strength and elongation as a function of alloy content for two series of alloys containing Fe, Mn and V respectively. One series, shown by solid lines numbered 1, 2 and 3, consists of conventional alloys of titanium with iron, manganese and vanadium, respectively, and containing .09% oxygen. The other series, shown in dotted lines numbers 4, 5 and 6, shows alloys of titanium with iron, manganese and vanadium, respectively, made in accordance with the present invention and containing .02% oxygen. The elongation curve, solid line numbered 7, represents the average elongation of the series of conventional alloys identified by lines 1, 2 and 3, while the elongation curve, solid line numbered 8, represents the average elongation of the series of low-oxygen alloys identified by lines 4, 5 and 6.

It will be seen that the maximum yield strength of alloys according to my invention is reached below 5% alloy content, and since ductility falls rapidly with increasing alloy content, the alloys showing desired strength at the lowest alloy content are generally most favorable.

Increasing oxygen in the alloys of my invention causes them to approach the YP-alloy content relationship shown in Figure 8 for conventional alloys. Within an oxygen content of more than .03%, the properties of the alloys are not significantly different from conventional alloys and this oxygen content is therefore regarded as the upper limit of my invention.

The maxima in the yield strength curves of the alloys of my invention as shown by the heavy lines of Figure 8 arise from a dispersion of a very small amount of alpha phase; with increasing content of beta stabilizers, the strengthening becomes that of solution only.

It will be understood that the analyses of the alloys to which I refer in this application are for the fabricated alloy and are for the average of a number of samples with a maximum variation of .005% oxygen. The elements present other than the specified oxygen and beta stabilizing elements are, in every case, less than .005%.

I have illustrated my invention with alloys containing a single beta stabilizing element. My invention encompasses alloys with two or more of the illustrated elements. In general, the effect of two or more alloying elements is additive so far as strengthening and the effect on ductility is concerned.

I have found, for example, that an alloy of 4% vanadium and 2% manganese with .01% oxygen provides a yield strength at 6% total alloy of 275,000 lbs. per square inch and an elongation of 18%. Such an alloy is but little affected by heat treatment since it is fully beta stabilized. The same alloy containing .07% oxy-

gen has a yield strength of about 140,000 lbs. and an elongation in 2" of 9%.

*Example I*

I made an alloy of titanium with 3% vanadium and 3% oxygen and the usual impurities in commercial titanium and vanadium. I comminuted the resulting brittle alloy to pieces having a largest dimension of 0.25 inch and smaller, and electro-refined it as follows: I placed the comminuted alloy in an annular foraminous steel basket and used this basket and contents as an anode in an electrolytic cell having a cylindrical cathode in the center of the annular anode basket. The cell was provided with an argon atmosphere and with means for separating the cathode and adhering material from the salt bath which latter was molten NaCl having dissolved therein 4.5% titanium as soluble chloride and 1% dissolved sodium. I passed a direct current through the cell at 25 amperes per lb. of comminuted anode material and 600 amperes per square inch on the cathode. A practically oxygen-free titanium-vanadium alloy containing about 3% vanadium was formed, attached to the cathode, at the rate of about .75 gram per ampere hour. The oxygen content of the alloy was only 0.005% oxygen.

After being melted in a vacuum arc furnace at a pressure of 1 micron, this alloy was formed into sheet by cold working and annealing at 800° C., the so-fabricated alloy contained .02% oxygen. The sheet had the following properties:

| Vickers Hardness | U.T.S.,<br>lbs./sq.in. | Y.S.,<br>lbs./sq.in. | Elong.,<br>Percent<br>in 2" |
|------------------|------------------------|----------------------|-----------------------------|
| 330-----         | 175,000                | 160,000              | 21                          |

I used this comminuted material as an anode exactly as in Example I, except that the bath contained 8% soluble zirconium chloride and 2% sodium.

The material adherent the cathode was a 3% vanadium-zirconium alloy containing 0.005% oxygen. This product was pressed into a consumable electrode, and was melted in an arc furance with a water-cooled copper hearth at 1 micron argon pressure. The resulting ingot was cold worked with vacuum annealing into bars. The resulting bars contained 0.025 oxygen and 2.9% vanadium. These bars had the following properties:

| Vickers Hardness | U.T.S.,<br>lbs./sq.in. | Y.S.,<br>(.1%<br>offset),<br>lbs./sq.in. | Elong.,<br>Percent<br>in 2" |
|------------------|------------------------|------------------------------------------|-----------------------------|
| 200-----         | 140,000                | 120,000                                  | 35                          |

*Example IV*

In this example, I proceeded as in Example II except that instead of .5% electrolytic manganese, I added 10% pure molybdenum.

The resulting bars had the following properties:

| Vickers Hardness | U.T.S.,<br>lbs./sq.in. | Y.S.,<br>lbs./sq.in. | Elong.,<br>Percent<br>in 2" |
|------------------|------------------------|----------------------|-----------------------------|
| 275-----         | 200,000                | 185,000              | 12                          |

*Example V*

In this example, I made three series of alloys by vacuum melting highly pure titanium and vanadium, and after fabricating by cold rolling and annealing in vacuum at 800° C., I obtained the following properties and analysis:

| Percent V | .02% Oxygen         |                   |                | .03% Oxygen |      |    | .07% Oxygen |      |    |
|-----------|---------------------|-------------------|----------------|-------------|------|----|-------------|------|----|
|           | U.T.S. <sup>1</sup> | Y.S. <sup>1</sup> | E <sup>1</sup> | U.T.S.      | Y.S. | E  | U.T.S.      | Y.S. | E  |
| 1-----    | 125                 | 90                | 30             | 70          | 55   | 28 | 55          | 45   | 20 |
| 2-----    | 140                 | 120               | 25             | 89          | 70   | 23 | 75          | 60   | 18 |
| 3-----    | 170                 | 155               | 20             | 125         | 100  | 17 | 90          | 70   | 15 |
| 4-----    | 185                 | 170               | 20             | 145         | 130  | 17 | 95          | 77   | 6  |
| 5-----    | 220                 | 210               | 20             | 180         | 15   | 15 | 100         | 82   | 0  |

<sup>1</sup> U.T.S.—in lbs./sq.in. Y.S.—lbs./sq.in. for .1% offset. E—Elongation, percent in 2".

*Example II*

In this example, I took crystal intergrowths of pure titanium analyzing 0.01% O<sub>2</sub> and substantially no other impurity. I prepared a consumable electrode by compacting this material with .5% electrolytic manganese. I melted this electrode in a water-cooled copper hearth arc furnace at .1 micron argon pressure. The resulting ingot was formed into bars by cold forging and vacuum annealing at 800° C. The resulting bars contained 0.02% oxygen and .47% manganese and had the following properties:

| Vickers Hardness | U.T.S.,<br>lbs./sq.in. | Y.S.,<br>(.1% off-<br>set),<br>lbs./sq.in. | Elong.,<br>Percent<br>in 2" |
|------------------|------------------------|--------------------------------------------|-----------------------------|
| 250-----         | 185,000                | 170,000                                    | 18                          |

*Example III*

In this example, I took a commercial zirconium alloy containing 3% vanadium and the customary amount of oxygen in solid solution, and comminuted it by milling.

These data are illustrated graphically in Figure 7 which shows the sharp change in relationship of yield strength and percent V in passing from the low oxygen contents of the present invention to the higher oxygen contents of the known art, e.g., .07% oxygen.

*Example VI*

In this example, I proceeded exactly as in Example I, except that I substituted chromium for vanadium in each and every operation. The result was a pure titanium-chromium alloy containing 1% Cr and, when fabricated, .02% oxygen.

The properties of the sheet alloy were:

| Vickers Hardness | U.T.S.,<br>lbs./sq.in. | Y.S.,<br>(.1% off-<br>set),<br>lbs./sq.in. | Elong.,<br>Percent<br>in 2",<br>percent |
|------------------|------------------------|--------------------------------------------|-----------------------------------------|
| 70 287-----      | 150,000                | 136,000                                    | 28                                      |

*Example VII*

In this example, I vacuum-melted pure zirconium with 2% iron. I cold worked and annealed at 800° C.

The resulting alloy was found to contain .03% oxygen, and had the following properties:

| U.T.S.<br>lbs./sq. in. | Y.S. (.1%<br>offset),<br>lbs./sq. in. | Elong.<br>in 2",<br>percent |
|------------------------|---------------------------------------|-----------------------------|
| 168,000                | 155,000                               | 22                          |

*Example VIII*

I proceeded as in Example I, except that I used as anode material comminuted zirconium alloy containing 2% manganese and 2% vanadium and 3% oxygen. The electrolyte was initially that of Example I. I carried out a preliminary electrolysis until the alloy being deposited on the cathode analyzed 46% Ti, 46% Zr, 4% V and 2% Mn. This alloy was melted in vacuum to produce an alloy containing equal parts of titanium and zirconium with 4% V, 2% Mn and .01% O<sub>2</sub>. This alloy was fabricated without oxygen absorption or other contamination and had the following properties when annealed in vacuum at 800° C.:

| U.T.S.,<br>p.s.i. | Y.P.,<br>p.s.i. | Elong.,<br>percent<br>in 2" |
|-------------------|-----------------|-----------------------------|
| 225,000           | 210,000         | 18                          |

### *Example IX*

In this example, I took needle-like crystal intergrowths containing 0.3% iron produced by electrorefining an iron-titanium alloy containing 5% iron according to Example I at a temperature of 1025° C. I melted these crystal intergrowths in an argon atmosphere at a pressure of 10 microns. The resulting ingot was coated with graphite and made a cathode in the refining bath of Example I, whereby to produce a continuous adherent coating of TiC thereon. I hot-rolled the ingot at 850° C. and scalped off .004 inch of surface. Analyses of the resulting fabricated alloy showed .025% oxygen, .3% iron, .0002 nitrogen and no other detectable impurities.

This alloy had the following properties after vacuum annealing at 900° C. and furnace cooling:

| U.T.S.,<br>p.s.i. | Y.S. (.1%<br>offset),<br>p.s.i. | Elongation |
|-------------------|---------------------------------|------------|
| 285,000           | 258,000                         | 5% in 2"   |

I claim:

1. A fabricated alloy, which is essentially a uniform solid solution on slow cooling from the beta range, consisting essentially of a metal selected from the group consisting of titanium and zirconium with from 1 to 10% of at least one beta stabilizing element and from 0.01 to not more than 0.03% of oxygen said alloy having a yield strength (1% offset), when slow-cooled from the beta range, of about 50,000 lbs./sq. in. greater at 1% beta

stabilizing agent and about 100,000 lbs. sq. in. greater at 10% beta stabilizing agent, with intermediate increases at intermediate amounts of beta stabilizing agent, than that of an alloy of the same metal composition but containing .05-.20% oxygen.

2. A fabricated titanium-vanadium alloy which is essentially a uniform solid solution on slow cooling from the beta range, said alloy consisting essentially of from about 1 to about 5% vanadium and from about 0.01 to not more than 0.03% oxygen in interstitial solid solution, balance substantially all titanium said alloy having a yield strength (.1% offset), when slow-cooled from the beta range, of about 50,000 p.s.i. greater at 1% alloy metal and about 100,000 p.s.i. greater at 5% alloy metal; with intermediate increases at intermediate amounts of alloy metal, than that of an alloy of the same metal composition but containing .05-.20% oxygen.

about 1 to about 5% vanadium and from about 0.01 to 10 not more than 0.03% oxygen in interstitial solid solution, balance substantially all titanium said alloy having a yield strength (.1% offset), when slow-cooled from the beta range, of about 50,000 p.s.i. greater at 1% alloy metal and about 100,000 p.s.i. greater at 5% alloy 15 metal, with intermediate increases at intermediate amounts of alloy metal, than that of any of the said

3. A fabricated titanium-manganese alloy which is essentially a uniform solid solution on slow cooling from

20 the beta range, said alloy consisting essentially of from about 1 to about 5% manganese and from about 0.01 to not more than 0.03% oxygen in interstitial solid solution, balance substantially all titanium said alloy having a yield strength (.1% offset), when slow-cooled from

25 the beta range, of about 50,000 p.s.i. greater at 1% alloy metal and about 100,000 p.s.i. greater at 5% alloy metal, with intermediate increases at intermediate amounts of alloy metal, than that of an alloy of the same metal composition but containing .05-.20% oxygen.

30 4. A fabricated titanium-iron alloy which is essentially a uniform solid solution on slow cooling from the beta range, said alloy consisting essentially of from about 0.1 to about 1.0% iron and from about 0.01 to not more than 0.03% oxygen in interstitial solid solution, balance 35 substantially all titanium.

5. A fabricated zirconium-iron alloy which is essentially a uniform solid solution on slow cooling from the beta range, said alloy containing from about 0.1 to about 1.0% iron and from about 0.01 to not more than 0.03% oxygen in interstitial solid solution, balance substantially all zirconium.

6. A fabricated alloy as defined in claim 1, in which the beta stabilizing element is molybdenum in an amount within the range 1 to 10%.

45 7. A fabricated alloy as defined in claim 1 having a total alloy content of beta stabilizing element of from 1 to 6% made up of vanadium and manganese in a proportion of at least 2 to 1.

**50 References Cited in the file of this patent**

UNITED STATES PATENTS

- |            |               |               |
|------------|---------------|---------------|
| Re. 24,013 | Jaffee et al. | May 31, 1955  |
| 2,596,485  | Jaffee et al. | May 13, 1952  |
| 2,622,023  | Frazier       | Dec. 16, 1952 |
| 2,754,203  | Vordahl       | July 10, 1956 |
| 2,754,204  | Jaffee et al. | July 10, 1956 |
| 2,754,205  | Jaffee et al. | July 10, 1956 |

#### OTHER REFERENCES

- 69 Transactions of ASM (Adenstedt et al.), vol. 44, pp. 990-1003, 1952. (Pages 990 and 991 relied on.)  
Metal Treatment and Drop Forging (Allen), pp. 245-252, June 1953. (Page 245 relied on.)  
ASM 1952 Preprint, No. 35, pp. 1-7, March 1953.

UNITED STATES PATENT OFFICE  
CERTIFICATE OF CORRECTION

Patent No. 2,920,957

January 12, 1960

William W. Gullett

It is hereby certified that error appears in the printed specification of the above numbered patent requiring correction and that the said Letters Patent should read as corrected below.

Column 8, line 38, claim 5, strike out "containing" and insert instead -- consisting essentially of --.

Signed and sealed this 7th day of June 1960.

(SEAL)

Attest:

KARL H. AXLINE  
Attesting Officer

ROBERT C. WATSON  
Commissioner of Patents